



US008377324B2

(12) **United States Patent**  
**Fairbourn**

(10) **Patent No.:** **US 8,377,324 B2**  
(b5) **Date of Patent:** **Feb. 19, 2013**

(54) **METHODS FOR REMOVING COATINGS  
FROM A METAL COMPONENT**

(75) Inventor: **David C. Fairbourn**, Sandy, UT (US)

(73) Assignee: **Acromet Technologies Inc.**, Sandy, UT (US)

(\*) Notice: Subject to any disclaimer, the term of this patent is extended or adjusted under 35 U.S.C. 154(b) by 892 days.

(21) Appl. No.: **12/415,492**

(22) Filed: **Mar. 31, 2009**

(65) **Prior Publication Data**

US 2009/0229636 A1 Sep. 17, 2009

**Related U.S. Application Data**

(63) Continuation-in-part of application No. 12/046,708, filed on Mar. 12, 2008, now Pat. No. 8,262,870, which is a continuation-in-part of application No. 11/423,363, filed on Jun. 9, 2006, now abandoned.

(60) Provisional application No. 60/689,482, filed on Jun. 10, 2005, provisional application No. 60/690,262, filed on Jun. 14, 2005.

(51) **Int. Cl.**

**C23F 1/00** (2006.01)

**C25F 1/00** (2006.01)

(52) **U.S. Cl.** ..... **216/95; 205/641; 216/7; 134/2; 134/38**

(58) **Field of Classification Search** ..... **205/641; 134/2, 38; 216/7, 95**

See application file for complete search history.

(56) **References Cited**

**U.S. PATENT DOCUMENTS**

3,335,087 A \* 8/1967 Keers, Jr. ..... 134/3  
4,268,397 A 5/1981 Horie et al.  
4,608,091 A 8/1986 Sullivan et al.  
4,746,369 A 5/1988 Sullivan et al.  
5,062,941 A 11/1991 Sue

|                   |         |                              |
|-------------------|---------|------------------------------|
| 5,232,619 A       | 8/1993  | Sue                          |
| 5,290,362 A       | 3/1994  | Sue                          |
| 6,294,072 B1      | 9/2001  | Fairbourn                    |
| 6,332,970 B1      | 12/2001 | Coffey                       |
| 6,428,683 B1      | 8/2002  | Jaworowski et al.            |
| 6,623,564 B2 *    | 9/2003  | Yamaguchi et al. .... 134/16 |
| 6,645,365 B2      | 11/2003 | Fairbourn et al.             |
| 6,837,985 B2      | 1/2005  | Fairbourn et al.             |
| 7,332,024 B2 *    | 2/2008  | Kool ..... 106/287.17        |
| 7,896,726 B1 *    | 3/2011  | Miller et al. ..... 451/2    |
| 2002/0108861 A1   | 8/2002  | Emesh et al.                 |
| 2003/0062271 A1   | 4/2003  | Kool et al.                  |
| 2004/0195110 A1   | 10/2004 | Emesh et al.                 |
| 2005/0164498 A1   | 7/2005  | Idé et al.                   |
| 2005/0199510 A1   | 9/2005  | Kochergin et al.             |
| 2005/0218010 A1 * | 10/2005 | Wang et al. ..... 205/677    |
| 2006/0027463 A1   | 2/2006  | Lavelle et al.               |
| 2007/0051619 A1   | 3/2007  | Mazur et al.                 |
| 2009/0302004 A1 * | 12/2009 | Manier et al. ..... 216/95   |

**FOREIGN PATENT DOCUMENTS**

WO WO 2007041998 A1 \* 4/2007

**OTHER PUBLICATIONS**

USPTO, Office Action issued in related U.S. Appl. No. 11/423,363 dated Dec. 23, 2009.

USPTO, final Office Action issued in related U.S. Appl. No. 11/423,363 dated Jun. 18, 2010.

U.S. Patent and Trademark Office, Office Action issued in U.S. Appl. No. 12/046,708 dated Sep. 2, 2011.

USPTO, final Office Action issued in related U.S. Appl. No. 12/046,708 dated Apr. 10, 2012.

USPTO, Notice of Allowance issued in related U.S. Appl. No. 12/046,708 dated Jun. 14, 2012.

\* cited by examiner

*Primary Examiner* — Nicholas A. Smith

(74) *Attorney, Agent, or Firm* — Wood, Herron & Evans, LLP

(57) **ABSTRACT**

Methods for removing coatings from metal components, such as metal components used in aircraft and other aerospace vehicles and the oil industry. The method may include removing an outer layer of a coating with a first stripping operation, removing an inner layer of the coating with a second stripping operation, and specifying an aqueous bath for either the first stripping process based upon an element in the outer layer or the second stripping process based upon an element in the inner layer.

**25 Claims, 2 Drawing Sheets**





FIG. 1



FIG. 2



FIG. 4



FIG. 3

## 1

METHODS FOR REMOVING COATINGS  
FROM A METAL COMPONENTCROSS-REFERENCE TO RELATED  
APPLICATIONS

This application is a continuation-in-part of application Ser. No. 12/046,708, filed Mar. 12, 2008, now U.S. Pat. No. 8,262,870, which is a continuation-in-part of application Ser. No. 11/423,363, filed on Jun. 9, 2006, now abandoned, which claims the benefit of U.S. Provisional Application No. 60/689,482, filed Jun. 10, 2005, and claims the benefit of U.S. Provisional Application No. 60/690,262, filed Jun. 14, 2005, the disclosure of each of which is hereby incorporated by reference herein in its entirety.

## BACKGROUND

The invention relates to stripping coatings from metal components and, more particularly, to methods for removing coatings from metal components used in aircraft and other aerospace vehicles, and the oil industry.

Aircraft landing gears include metal components, such as inner and outer cylinders, axles, pins, and actuators, formed from high strength structural materials like steel alloys. The metal components of aircraft landing gears, as well as the metal segments or components of exhaust augmentor flaps or turkey feathers and compressor blades found in aircraft engines, are often encapsulated or at least partially covered by a coating to provide a beneficial effect, such as corrosion resistance. For example, a coating, such as WCCo CrC/NiCr, or (WC/CoCr), may be applied to these metal components by, for example, a plasma spraying technique or by a high velocity oxygen fuel (HVOF) thermal spray process. The coatings are also used to coat shafts, gear boxes, and other wear parts in other industries, such as the oil industry.

Landing gears and exhaust augmentor flaps, as well as compressor blades and other rotating engine parts, are periodically removed from aircraft to inspect the material forming the metal components for stress corrosion, cracking, or other evidence of a condition that could lead to a field failure while in service. The inspection requires that the coating be stripped so that the coating does not interfere with the inspection process. For example, a porous coating may restrict the ability of a penetrant to reach the underlying structural material. If the component passes inspection, a new coating is applied to the metal component before the landing gear or exhaust augmentor flap is returned to service.

Conventional processes for stripping coatings suffer from various deficiencies. For example, a reverse plating process using an aqueous bath containing tartaric acid may be used to remove tungsten-containing coatings. However, this particular reverse plating process is expensive and slow. Aqueous baths containing acids may cause metal components formed from high strength steel alloys to be susceptible to hydrogen ion embrittlement. Embrittled metal components may become susceptible to damage from shock. Although residual trapped hydrogen in the stripped metal components may be removed by a low temperature bake, the required length of the bake slows process throughput.

Nevertheless, there is a need for improved apparatus, methods, and compositions to efficiently remove coatings from metal components used in aircraft and other aerospace vehicles.

## SUMMARY

The invention provides, in one aspect, an improved method for efficiently removing a coating from a metal component

## 2

used in aircraft and other aerospace vehicles that measures an oxygen concentration of an aqueous bath, which contacts at least a portion of the metal component, and adds an amount of the active oxygen chemical source to the aqueous bath if the measured oxygen concentration differs from a reference oxygen concentration. By virtue of the foregoing, there is provided a method for removing coatings in which the active oxygen content of the aqueous bath is tracked and adjusted to optimize removal as the composition or chemistry of the aqueous bath is altered by the coating-removal process.

The invention provides, in another aspect, an improved apparatus that includes a first sensor in fluid communication with an aqueous bath, which contacts at least a portion of the metal component, and adapted to measure an oxygen concentration of the aqueous bath. The apparatus further includes a control system responsive to output signals indicative of the oxygen concentration supplied from the first sensor to cause an additional amount of a first aqueous bath component to be added to the aqueous bath. Advantageously, the sensor and control system cooperate to adjust the composition or chemistry of the aqueous bath if the measured value of the oxidation reduction potential deviates from a reference value, which maintains the efficiency of the stripping process as the coating-removal process modifies the composition or chemistry of the aqueous bath. The use of the oxygen sensor may improve the ability of the control system to respond to measured variations in the active oxygen content with relatively high concentrations of a ligand, such as citric acid, in the aqueous bath and, in particular, with a concentration of the ligand to endow the bath with a relatively low pH value, such as pH values of about 1.75 to about 2.75.

The invention provides, in another aspect, an improved method for efficiently removing a coating from a metal component used in aircraft and other aerospace vehicles that measures an oxidation reduction potential of an aqueous bath, which contacts at least a portion of the metal component, and adds an amount of the active oxygen source to the aqueous bath to increase the oxidation reduction potential if the measured oxidation reduction potential differs from a reference oxidation reduction potential. By virtue of the foregoing, there is provided a method for removing coatings in which the active oxygen content of the aqueous bath is tracked and adjusted to optimize removal as the composition or chemistry of the aqueous bath is altered by the coating-removal process.

The invention provides, in another aspect, an improved method for efficiently removing a coating from a metal component used in aircraft and other aerospace vehicles by adjusting the composition of an aqueous bath, which contacts at least a portion of the metal component, to maintain the pH value between about 7.0 and about 9.0. By virtue of the foregoing, there is provided a method for removing coatings in which the pH value of the aqueous bath is adjusted so that the substrate of the metal component is not damaged by chemical attack by the aqueous bath. Another description of this process is to passivate the substrate. The adjustments may be made in response to changes in the composition or chemistry of the aqueous bath resulting from the coating-removal process.

The invention provides, in another aspect, an improved apparatus that includes a first sensor in fluid communication with an aqueous bath, which contacts at least a portion of the metal component, and adapted to measure an oxidation reduction potential of the aqueous bath. The apparatus further includes a control system responsive to output signals indicative of the oxidation reduction potential supplied from the first sensor to cause an additional amount of a first aqueous bath component to be added to the aqueous bath. Advantage-

geously, the sensor and control system cooperate to adjust the composition or chemistry of the aqueous bath if the measured value of the oxidation reduction potential deviates from a reference value, which maintains the efficiency of the stripping process as the composition or chemistry of the aqueous bath is modified by the coating-removal process.

In another aspect, the invention provides compositions for an aqueous bath used to remove at least a portion of a coating from a metal component.

In one embodiment, the composition comprises water, hydrogen peroxide ( $H_2O_2$ ), and a ligand selected from the group consisting of citric acid ( $C_6H_8O_7$ ), oxalic acid ( $C_2H_2O_4$ ), tartaric acid ( $C_4H_6O_6$ ), formic acid ( $CH_2O_2$ ), or glucose (6-hydroxymethyl) oxane-2,3,4,5-tetrol). The ligand is present with a concentration sufficient to provide a pH value of about 1.75 to about 2.75. These pH values of the composition may be beneficial if the coating is WCCo.

As understood by a person having ordinary skill in chemistry, a ligand is an atom, ion, molecule, or a functional group that generally donates one or more of its electrons through a coordinate covalent bond to, or shares its electrons through a covalent bond, or through a pi-bond, with one or more central atoms or ions. These latter ligands act as a Lewis base.

In another embodiment, the composition comprises water, an active oxygen source selected from the group consisting of sodium perborate tetrahydrate ( $NaBO_3 \cdot 4H_2O$ ), sodium perborate monohydrate ( $NaBO_3 \cdot H_2O$ ) prepared by dehydrating sodium perborate tetrahydrate, sodium percarbonate ( $Na_2CO_3 \cdot 1\frac{1}{2}H_2O_2$ ), boric acid ( $H_3BO_3$ ), and combinations thereof, and a ligand selected from the group consisting of citric acid ( $C_6H_8O_7$ ), oxalic acid ( $C_2H_2O_4$ ), tartaric acid ( $C_4H_6O_6$ ), formic acid ( $CH_2O_2$ ), glucose (6-hydroxymethyl)oxane-2,3,4,5-tetrol), and combinations thereof. A pH value of the composition is within a range of about 7.0 to about 9.0. If coating to be stripped using the composition contains nickel or chromium to impart corrosion resistance in acidic stripping solutions, then this composition may be particularly beneficial for stripping such coatings.

In another embodiment, a method is provided for removing a coating including an outer layer and an inner layer between the outer layer and an underlying metal component. The method includes removing the outer layer of the coating with a first stripping operation, removing the inner layer of the coating with a second stripping operation, and specifying an aqueous bath for either the first stripping process or the second stripping process based respectively upon an element in the outer layer or an element in the inner layer.

In another embodiment, a method is provided for removing a coating including an outer layer composed of aluminum polyester resin, an inner layer, and an intermediate layer composed of Ni between the outer layer and inner layer. The method includes removing the outer layer of the coating with an aqueous bath containing NaOH, removing the intermediate layer with an aqueous bath containing dilute nitric acid, and, after the outer layer and the intermediate layer are removed, removing the inner layer of the coating. The Ni layer serves as a bond coat applied over the inner layer to improve the adhesion of the aluminum polyester layer.

These and other objects and advantages of the invention shall be made apparent from the accompanying drawings and description thereof.

#### BRIEF DESCRIPTION OF THE DRAWINGS

The accompanying drawings, which are incorporated in and constitute a part of this specification, illustrate an embodiment of the invention and, together with a general

description of the invention given above, and the detailed description of the embodiment given below, serve to explain the principles of the invention.

FIG. 1 is a highly schematic, not to scale view of a metal component bearing a coating to be stripped in accordance with the invention;

FIG. 2 is a cross-sectional view of an edge portion of the metal component and coating of FIG. 1;

FIG. 3 is a diagrammatic view of an apparatus for stripping the coating from the metal component of FIG. 1 in accordance with an embodiment of the invention; and

FIG. 4 is a cross-sectional view similar to FIG. 2 after the coating is stripped from the metal component.

15

#### DETAILED DESCRIPTION

With reference to FIGS. 1-4, the invention provides for the removal or stripping of a coating 10 from a metal component 12 representative of a metal component of an aircraft landing gear. The coating 10 may be composed of tungsten carbide cobalt (WCCo), CrC/NiCr, tungsten carbide cobalt-chromium (WC/CoCr), or another material, such as a material characteristic of plasma-sprayed coatings applied by high-velocity oxy-fuel (HVOF) techniques, air plasma spray techniques, cold spray techniques, combustion wire techniques, cold spray techniques, combustion wire techniques, arc spray techniques, arc wire spray techniques, or combustion powder techniques. A substrate 14 of the metal component 12 is formed from a structural material, such as a high strength structural steel alloy (e.g., ASI 4140 and ASI 4340), that differs in composition from the material forming the coating 10. The coating 10 is applied to an original surface 16 of substrate 14. If the coating 10 is completely or almost completely removed, all or a portion of the original surface 16 is revealed.

The landing gear is understood to include additional metal components, in addition to the illustrated metal component 12, that would benefit from coating stripping as described herein. The invention also contemplates that the metal component 12 may consist of an assembly of several individual components that are simultaneously removed by a single stripping operation. Exemplary metal components 12 of a landing gear include, but are not limited to, the inner and outer cylinders, axles, pins, actuators such as hydraulic actuators, and assemblies of these and other individual components. The assemblies may include additional components (not shown) that are uncoated by the coating 10.

Metal component 12 may also comprise an exhaust augmentor flap segment or component normally used in service near the exhaust outlet of a jet engine. The substrate 14 of this type of metal component 12 may be formed from a material, such as titanium, Inconel 718 (a nickel based superalloy), niobium, or another suitable material as understood by a person having ordinary skill in the art.

In accordance with the principles of the various embodiments of the invention, the coating 10 is stripped from at least a portion of the metal component 12 to reveal the original surface 16 of the substrate 14. Metal component 12 is associated with an aqueous bath 18, such as by being fully or at least partially immersed in a solution-filled tank or container 20 of a stripping apparatus 25 as shown in FIG. 3. Only a portion of the metal component 12 may be contacted or wetted by the aqueous bath 18 so that the coating 10 is only removed from the wetted portion and remains substantially intact on the unwetted regions after the stripping process. It is contemplated that residual coating 10 may remain on a portion of the metal component 12. The invention contemplates

60

65

that the stripping process removing the coating 10 may also remove or mill away a minor thickness of the substrate 14 of the metal component 12 after the coating 10 is at least partially removed. Preferably, the substrate 14 is undamaged by the stripping operation or any damage suffered is negligible.

Container 20 may be made of any material appropriate for the particular application, such selection being within the ordinary skill of one in the art, and for example, may comprise plastic or metal, such as stainless steel. The container 20 is dimensioned and the volume of solution constituting aqueous bath 18 is sufficient to receive and fully immerse the metal component 12. The metal component 12, which is part of an assembly designed to support the massive weight of an aircraft under the violent impact and shock of landing, is understood by persons of ordinary skill in the art to be dimensionally large and bulky. Consequently, removing coating 10 from component 12 requires a relatively large container 20 and a relatively large volume of solution in aqueous bath 18. Consequently, container 20 is of a type that would not be used in small-scale laboratory experiments.

For example, container 20 may be sized to hold a bath 18 of up to 9000 gallons (34,000 liters) of solution for stripping metal components 12 that may approach about 15 feet (about 4.572 meters) in length and about 1 foot (about 0.3048 meter) in diameter. Alternatively, if the metal component 12 originates from an exhaust augmentor flap, container 20 may be sized to hold a bath 18 of up to 40 liters (1.413 cubic feet) of solution for stripping metal components 12 of an exhaust augmentor flap that may approach about 19 inches (about 48.26 centimeters) in length and about 8 inches (about 20.32 centimeters) or so in width.

The aqueous bath 18 may be at room temperature, which varies according to the environment, but it is typically between about 55° F. and about 105° F. (about 13° C. to about 41° C.). In one embodiment, the aqueous bath 18 may be maintained at about 95° F. (32° C.) or less. However, in certain embodiments of the invention, the aqueous bath 18 may be warmed to higher temperatures, if desired, to accelerate the stripping process. This may be achieved by adding a heat source (not shown) adapted to heat the electrolyte in aqueous bath 18. In other embodiments of the invention and as described hereinafter, the aqueous bath 18 may also be chilled to limit the temperature.

With reference to FIG. 3, the stripping apparatus 25 further includes a counter electrode 22 associated with aqueous bath 18, such as by being contacted or immersed in container 20 with metal component 12. The counter electrode 22 may be formed from graphite or from other materials such as stainless steel 304, gold, platinum, or Hastelloy C-276. Metal component 12 has a first natural standard electrode potential  $E^\circ$ , and counter electrode 22 has a second natural standard electrode potential  $E^\circ$  greater than the  $E^\circ$  of the metal component 12. Counter electrode 22 and metal component 12 are DC coupled by an electrical path or coupling, as exemplified by a wire 24, to establish a circuit. The surface area of the counter electrode 22 may be approximately equal to the surface area of the metal component 12. Alternatively, the counter electrode 22 may be introduced as a liner inside the container 20, and the metal component 12 may be placed or otherwise rest directly on the liner to establish the DC coupling with the counter electrode 22.

The standard electrode potential,  $E^\circ$ , which is expressed in volts, is defined as the potential of an element immersed in a solution of its ions at unit activity.  $E^\circ$  may be measured by electrochemical impedance spectroscopy (EIS). A driving or electromotive force (EMF) results from the relative potential forces of the two dissimilar electrodes (i.e., the metal com-

ponent 12 and the counter electrode 22). The greater the magnitude of the differential between the  $E^\circ$  values of the metal component 12 and the counter electrode 22, the greater the EMF produced, and thus a faster and more effective stripping of the coating 10 may be obtained.

Although not wishing to be bound by theory, the use of the counter electrode 22 is believed to eliminate or significantly reduce the risks associated with hydrogen embrittlement of the metal component 12 by reducing hydrogen infiltration from the aqueous bath 18 into the metal component 12. The metal component 12 operates as an anode during stripping, while the counter electrode 22 operates as the cathode on which substantially all cathodic activity occurs. The surface 16 of metal component 12 surrenders electrons by virtue of the  $E^\circ$  differential between the metal component 12 and the counter electrode 22.

The stripping process is continued until the coating 10 is at least partially removed and, preferably, completely removed from metal component 12 to expose original surface 16, as is apparent in FIG. 4. The solution in bath 18 may be stirred or otherwise agitated to enhance the removal rate of the coating 10. For example, an ultrasonic probe 26 may be inserted into the aqueous bath 18 to produce shock waves that agitate the solution constituting the aqueous bath 18, although the frequency does not have to be ultrasonic to be effective and sonic frequencies may be useful. Other examples of agitating mechanisms are a mechanical agitator with, for example, a bladed impeller or a pump (not shown) that adds and extracts solution from the tank to thereby agitate the aqueous bath 18. The pumped solution may be filtered to remove particulates that accumulate in the aqueous bath 18. The pumping may be continuous or intermittent and the filtered solution may be returned to the container 20 through a sparger that injects the returned solution with jets oriented to direct flows generally toward the metal component 12. As described hereinafter, the pumped solution may also be chilled to control the temperature of the aqueous bath 18.

With continued reference to FIG. 3, an optional external power source 28 may be placed in the circuit coupling the metal component 12 and counter electrode 22 to add an additional EMF that may, for example, be in the range of one (1) to six (6) volts. The additional EMF modifies the  $E^\circ$  differential between the metal component 12 and the counter electrode 22. A positive cathode of the optional power source 28 is DC coupled to the metal component 12, and a negative anode of the optional power source 28 is DC coupled to the counter electrode 22. The power source 28 supplies an external voltage in the negative sense from the counter electrode 22 to the metal component 12 that expands the effect of the natural  $E^\circ$  differential. The presence of the negative potential is believed to advantageously increase the removal rate of the coating 10 while the metal component 12 is contacted by or immersed in the aqueous bath 18 and DC coupled with the counter electrode 22. In particular, the use of power source 28 may be particularly beneficial for increasing the removal rate of WCCoCr, wherein the chromium is only 4% of the chemistry of the coating 10.

In one aspect of the invention, the electrolyte in aqueous bath 18 may be a dilute aqueous solution consisting of a mixture of deionized water ( $H_2O$ ), a source of active oxygen such as hydrogen peroxide ( $H_2O_2$ ), and a substance that behaves as a ligand for removed metal. The ligand may be an acid selected from citric acid ( $C_6H_8O_7$ ), oxalic acid ( $C_2H_4O_4$ ), tartaric acid ( $C_4H_6O_6$ ), glucose (6-(hydroxymethyl)oxane-2,3,4,5-tetrol), or formic acid ( $CH_2O_2$ ). A person having ordinary skill in the art understands that a ligand is an atom, ion, or molecule that donates one or more of its

electrons through a coordinate covalent bond to, or shares its electrons through a covalent bond with one or more central metal atoms or ions to form a complex.

The measured oxidation reduction potential or oxygen concentration of the aqueous bath **18** provides a qualitative measure of the oxidation power of the aqueous bath **18**. The oxidation power provides an indication of the solution's ability to oxidize the constituent material of the coating **10**. The measured oxidation reduction potential or oxygen concentration is related to the concentration of active oxygen in the aqueous bath **18** and the activity or strength of the source of active oxygen. As the coating **10** is removed, active oxygen is consumed in the process, which causes the measured oxidation reduction potential or oxygen content of the aqueous bath **18** to change in a predictable manner that can be correlated with the concentration of active oxygen in the aqueous bath **18**. The pH of the aqueous bath **18**, as well as the concentration of ligand that is not bound with metal ions from the coating **10** and dissolved in bath **18**, also changes during the coating removal process.

In one specific embodiment of the invention, the aqueous bath **18** includes a volume of hydrogen peroxide sufficient to provide a level of about 3 percent of the total solution volume, about 2 grams (about 0.07055 ounce) of citric acid per liter of solution, and the rest water. In another specific embodiment of the invention, the aqueous bath **18** includes a total volume of 60 gallons (227.1 liters), about 0.00833 volume percent of hydrogen peroxide (i.e., about 0.5 gallons (about 1.893 liters)), about 120 grams (about 4.233 ounces) of citric acid per liter of solution, and the rest water. In another embodiment, the composition of the aqueous bath **18** contains hydrogen peroxide at a level of about 1 wt. % to about 32 wt. %, with the balance being water and ligand.

Although not wanting to be bound by theory, the use of citric acid or another of the described acids or functionally-equivalent acids is believed to enhance the removal of metal from the coating **10** by operating as a chelating agent that binds the metal ions removed from metal component **12** by the hydrogen peroxide and, on that basis, to enhance the removal rate for stripping coating **10** from metal component **12**.

The stripping apparatus **25** may include a probe or sensor **30** capable of measuring the oxidation reduction potential of the aqueous bath **18** during the stripping process. Sensor **30** may be any suitable oxidation reduction potential sensor such as, for example, an electrochemical-type sensor. In particular, sensor **30** may comprise an electrode with a measuring half cell comprised of platinum metal immersed in the aqueous bath **18** and sealed a reference half cell to which the platinum half cell is referenced. Although sensor **30** is depicted as positioned inside the container **20** and wetted by bath **18**, sensor **30** may alternatively be a non-contact sensor otherwise positioned. Sensor **30** generates output signals that correspond to, or are proportional to, successive measurements of the oxidation reduction potential of aqueous bath **18**.

Alternatively, sensor **30** may be an oxygen sensor that is configured to directly detect the concentration of oxygen dissolved in the solution constituting the aqueous bath **18**. In one embodiment, the sensor **30** may be an electrode-type oxygen sensor that operates by an electrochemical mechanism. The electrode-type oxygen sensor **30** includes a cathode and an anode that are submersed in the aqueous bath **18**. Oxygen enters the electrode-type oxygen sensor **30** through a permeable membrane by diffusion from the aqueous bath **18**, and is reduced at the cathode, creating a measurable electrical current that is communicated from the sensor **30** to the control system **34**, as described below. The electrical current is pro-

portional to the oxygen concentration in the bath **18**. In an alternative embodiment, the sensor **30** may be an optical-type oxygen sensor that optically measures the oxygen concentration. Typically, the optical-type oxygen sensor **30** will include an optical cable and a fluorescent film attached to the tip of the optical cable. The fluorescence from the fluorescent film, which is contingent on the oxygen concentration in the aqueous bath **18**, is analyzed by the control system **34** as indicative of the oxygen content.

10 The stripping apparatus **25** may also include a probe or sensor **31** capable of measuring the pH of the aqueous bath **18** during the stripping process. The pH sensor **31** may be any suitable pH sensor, such as a device having a working electrode and a reference electrode. Although pH sensor **31** is 15 depicted as positioned inside the container **20** and wetted by bath **18**, pH sensor **31** may alternatively be a non-contact sensor otherwise positioned. Sensor **31** generates output signals that correspond to, or are proportional to, successive measurements of the pH of aqueous bath **18**. As understood 20 by a person of ordinary skill in the art, the pH is a measure of the activity of hydrogen ions ( $H^+$ ) in the aqueous bath **18** and, therefore, the acidity or alkalinity. The pH value, which is a dimensionless number between 0.0 and 14.0, indicates 25 whether a solution is acidic ( $pH < 7$ ), neutral ( $pH = 7$ ), or basic/alkaline ( $pH > 7$ ).

With continued reference to FIG. 3, the sensor **30** and pH sensor **31** are coupled electrically with a control system **34** of the stripping apparatus **25** by communication links **32**, **33**, respectively. The communication links **32**, **33** may be constituted by a cable or wire, a radiofrequency (RF) link, or an infrared (IR) link. The output signals generated by the sensor **30** are directed over the communication link **32** to the control system **34**. Similarly, the output signals generated by the pH sensor **31** are directed over the communication link **33** to the control system **34**. The output signals from sensors **30**, **31** may be provided to the control system **34** at various different time intervals between successive measurements as required to maintain control over the composition of the solution forming the aqueous bath **18**. The output signals may be periodically, aperiodically, or continuously generated in response to the successive measurements, but are repeatedly measured without user intervention and supplied as feedback to the control system **34** for responding to the generated output signals.

45 Control system **34** is electrically coupled with an active oxygen source supply **38** of the stripping apparatus **25** over a communications link **40**, such a wire, a radiofrequency (RF) link, or an infrared (IR) link. The active oxygen source supply **38** includes a valve or flow control device **42** that the control system **34** can command to open and close for adding additional amounts **43** of the active oxygen source to the aqueous bath **18**. The active oxygen source supply **38** is a conventional structure that includes a bulk supply of the active oxygen source and any additional components as understood by a 50 person of ordinary skill in the art required for holding and transferring such substances.

Control system **34** is also electrically coupled with a ligand supply **48** of the stripping apparatus **25** over a communications link **50**, such a wire, a radiofrequency (RF) link, or an infrared (IR) link. The ligand supply **48** includes a valve or flow control device **52** that the control system **34** can command to open and close for adding additional amounts **53** of the ligand to the aqueous bath **18**. The ligand supply **48** is a conventional structure that includes a bulk supply of the ligand and any additional components as understood by a person of ordinary skill in the art required for holding and transferring such substances.

Control system 34 relies on a software algorithm and/or user input to respond to electrical signals supplied from sensor 30. Specifically, control system 34 may respond to a change (e.g., deficiency) in the amount of the source of active oxygen, as indicated by successive output signals representative of the measured oxidation reduction potential or oxygen concentration supplied from sensor 30, by causing additional amounts 43 of the active oxygen source to be transferred from the active oxygen source supply 38 through a transfer pathway 36 to the aqueous bath 18. A person of ordinary skill in the art will appreciate that other types of fluid transfer pathways 36 may be established, such as piping (not shown) extending from the active oxygen source supply 38 through the wall of the container 20. In the illustrated embodiment, the transfer pathway 36 is illustrated as introducing added amounts 43 of the active oxygen source at a location proximate to the sensor 30. However, the invention is not so limited as the transfer pathway 36 may introduce these additional amounts 43 of the active oxygen source at other locations so long as the added amounts are contained inside of container 20.

The control system 34 of the stripping apparatus 25 may compare the measured oxidation reduction potential or oxygen concentration as indicated by the sensor 30 with a reference oxidation reduction potential or oxygen concentration. Based upon the comparison, the control system 34 may instruct the active oxygen source supply 38 to add an amount 43 of the source of active oxygen to the aqueous bath 18 effective to increase the oxidation reduction potential. The oxidation reduction potential or oxygen concentration of the aqueous bath 18 may be increased to a measured value comparable or equal to the reference value. The control system 34 may regulate the rate of addition of the active oxygen source to maintain the measured oxidation reduction potential or oxygen concentration within an effective range for at least partially removing the coating 10 from the contacted portion of the metal component 12.

Control system 34 likewise relies on a software algorithm and/or user input to respond to electrical signals supplied from sensor 31. Specifically, control system 34 may respond to a change in the pH of aqueous bath 18, as indicated by successive output signals representative of the measured pH supplied from sensor 31, by causing additional amounts 53 of the ligand to be transferred from the ligand supply 48 through a transfer pathway 54 to the aqueous bath 18. A person of ordinary skill in the art will appreciate that other types of fluid transfer pathways 54 may be established, such as piping (not shown) extending from the ligand supply 48 through the wall of the container 20. In the illustrated embodiment, the transfer pathway 54 is illustrated as introducing added amounts 53 of the ligand at a location remote from the sensor 31. However, the invention is not so limited as the transfer pathway 54 may introduce these additional amounts 53 of the ligand at other locations so long as the added amounts are contained inside of container 20.

The control system 34 of the stripping apparatus 25 may compare the measured pH as indicated by the sensor 31 with a reference pH. If the measured pH differs from the reference pH, the control system 34 may instruct the ligand supply 48 to add an amount of the ligand to the aqueous bath 18 effective to decrease (or increase) the pH. The pH of the aqueous bath 18 may be increased to a measured pH value comparable or equal to the reference pH value. The control system 34 may regulate the rate of addition of the ligand to maintain the measured pH value within an effective range for at least partially removing the coating 10 from the contacted portion of the metal component 12 without attacking or damaging the substrate 14.

The invention contemplates that the active oxygen source and/or ligand may be added to the aqueous bath 18 as a solid, rather than in a liquid form as depicted in FIG. 3.

The stripping apparatus 25 may optionally include a recirculation system with a pump 56 and a chiller 58 that cooperate to regulate the temperature of the aqueous bath 18 in container 20. A temperature sensor 57, which is connected with the control system 34 by a communication link similar to communication links 32, 33, may measure the temperature of the solution in the aqueous bath 18 and provide output signals representing the temperature as feedback to the control system 34. The control system 34 can use the temperature feedback for closed-loop control of the operation of chiller 58 so as to maintain the temperature of the aqueous bath 18 at or below a maximum temperature, or with a temperature range.

The ability of regulate the temperature of the aqueous bath 18 may be beneficial for use with a bath chemistry that contains hydrogen peroxide ( $H_2O_2$ ) as the active source of oxygen and citric acid as the ligand. In one embodiment of the invention, the temperature of the aqueous bath 18 is regulated such that the bath temperature is kept at about 95° F. (32° C.) or less, which limits the loss of active oxygen from the hydrogen peroxide in the bath 18 to the ambient atmosphere surrounding the stripping apparatus 25. This permits the pH value of the aqueous bath 18 to be maintained at about 2.0, or lower, during the operation of the stripping apparatus 25 and by additions of citric acid sufficient to establish this pH value, which may increase the efficiency of removing coatings 10 of certain compositions. In another embodiment, the pH of the aqueous bath 18 is maintained in a range of about 1.75 to about 2.75 and the temperature is controlled to avoid excess peroxide disassociation. If not temperature controlled while stripping, the concentration of hydrogen peroxide in the aqueous bath 18 in combination with the low pH value may also cause the temperature to rise above about 95° F. and, as a result, prompt an uncontrolled loss of active oxygen from the bath 18. In another embodiment, the temperature of the aqueous bath 18 may be maintained by temperature control in a range between about 30° C. (85° F.) and about 33° C. (91° F.).

With reference to FIG. 3, the stripping apparatus 25 may optionally include a base supply 62 that is adapted to transfer amounts 60 of a base substance through a transfer pathway 64 to the aqueous bath 18. A person of ordinary skill in the art will appreciate that other types of fluid transfer pathways 64 may be established, such as piping (not shown) extending from the base supply 62 through the wall of the container 20. Control system 34 is electrically coupled with the base supply 62 of the stripping apparatus 25 over a communications link 66, such as a cable or wire, a radiofrequency (RF) link, or an infrared (IR) link. The base supply 62 includes a valve or flow control device 68 that the control system 34 can command to open and close for adding additional amounts 60 of the base to the aqueous bath 18. Base supply 62 is a conventional structure that includes a bulk supply of the base and any additional components as understood by a person of ordinary skill in the art required for holding and transferring such substances. The base supply 62 may be omitted if the composition of the aqueous bath 18 lacks a base/alkaline substance.

The control system 34 of the stripping apparatus 25 may compare the measured pH as indicated by the sensor 31 with a reference pH. If the measured pH differs from the reference pH, the control system 34 may instruct the base supply 62 to add an amount of the base to the aqueous bath 18 effective to decrease the pH. The pH of the aqueous bath 18 may be decreased to a measured pH value comparable or equal to the reference pH value by instructing the base supply 62 to add amounts 60 of the base to the aqueous bath 18. The control system 34 may regulate the rate of addition of the base to maintain the measured pH value within an effective range for

## 11

at least partially removing the coating **10** from the contacted portion of the metal component **12** without attacking or damaging the substrate **14**.

The original surface **16**, when exposed after the coating **10** is stripped, may be susceptible to damage from, for example, corrosion. To that end and in certain embodiments of the invention, amounts of the base substance may be added to the aqueous bath **18** sufficient to adjust the pH to a pH value that prevents damage to the metal component **12** after the coating **10** is removed. Damage is prevented without significantly altering the stripping rate or, at the least, only altering the stripping rate within tolerable limits. The added amount **60** of the base is be sufficient to adjust the pH to a pH value greater than about 7.0 but less than, or equal to, 8.0. This maintains the solution pH at a neutral to slightly basic/alkaline value. In another embodiment, the pH of the aqueous bath **18** is maintained at a pH value in the range of about 7.0 to about 9.0.

An exemplary chemical substance useful for adjusting the pH is sodium hydroxide (NaOH), which is available commercially in various solid forms, e.g., pellets, sticks, or chips, and in water solutions of various concentrations, and is commonly known as caustic soda, lye, or sodium hydrate. The ability to adjust the pH may be particularly advantageous for preventing corrosion, which may have the form of rust, of metal components **12** in which the substrate **14** is formed from a material susceptible to corrosion. Exemplary corrosion-susceptible materials for substrate **14** include, but are not limited to, 4140 and 4340 stainless steels.

For operation at these pH values, the source of active oxygen in the aqueous bath **18** may be a chemical compound or substance such as sodium perborate tetrahydrate (NaBO<sub>3</sub>.4H<sub>2</sub>O), sodium perborate monohydrate (NaBO<sub>3</sub>.H<sub>2</sub>O) prepared by dehydrating sodium perborate tetrahydrate, sodium percarbonate (Na<sub>2</sub>CO<sub>3</sub>.1½H<sub>2</sub>O<sub>2</sub>), boric acid (H<sub>3</sub>BO<sub>3</sub>), mixtures of these chemical compounds or substances, or the like. In one embodiment, the source of active oxygen may be present at a level of from 1% to 30% by weight of the composition. The chemical substance supplying the active oxygen may undergo dissociation or hydrolysis in contact with water, producing active oxygen in the aqueous bath **18**. The pH of the aqueous bath **18** may be adjusted using the alternative active oxygen source to a pH value greater than about 7.0 and less than, or equal to, 8.0 without concerns regarding the evaporative loss of hydrogen peroxide. Replacing hydrogen peroxide with a different active oxygen source eliminates the difficulties associated with the expected loss of hydrogen peroxide from the aqueous bath **18** at elevated pH and temperature values.

In one embodiment, use of NaBO<sub>3</sub>.4H<sub>2</sub>O, NaBO<sub>3</sub>.H<sub>2</sub>O, Na<sub>2</sub>CO<sub>3</sub>.1½H<sub>2</sub>O<sub>2</sub>, or H<sub>3</sub>BO<sub>3</sub> may permit coating **10** to be simultaneously removed from multiple metal components **12** placed in the aqueous bath **18** in a situation in which different components **12** have coatings **10** of different compositions. For example, the composition of the coating **10** on one metal component **12** may be WCCo and the composition of the coating **10** on another metal component **12** may be CrC/NiCr. Yet, the stripping conditions in the stripping apparatus **25** promote the efficient stripping of the two different types of coating **10**. This ability permits coatings **10** of different compositions to be simultaneously stripped from batches of metal components **12** without actually determining the specific coating compositions. In addition, coating **10** may include material of one composition, such as WCCo, on one region of the metal component **12** and material with another composition, such as CrC/NiCr, on another region of the metal component **12**, yet the stripping conditions in the stripping apparatus **25** promote efficient stripping. In one embodiment of the invention, the temperature of the aqueous bath **18** is regulated such that the temperature of the aqueous bath **18** is maintained in a range at about 50° C. (122° F.) to about 65° C.

## 12

(149° F.), which may promote faster coating removal than for temperatures less than about 50° C.

In one embodiment, the chemistry of the solution in the aqueous bath **18** may include sodium citrate, sodium carbonate and sodium perborate with each component present at about one-third molar concentration for each component. In another embodiment, the chemistry of the solution in the aqueous bath **18** may include about ⅔ molar sodium citrate, 0.2 molar or 0.1 molar sodium perborate, and about ⅓ sodium carbonate. The pH may be adjusted by additions of sodium carbonate to maintain the pH in a range of about 7.0 to about 9.0.

In accordance with this embodiment, the control system **34** may respond to a change in the pH of aqueous bath **18** occurring during the coating removal process, as indicated by successive output signals representative of the measured pH supplied from sensor **31**, by causing amounts **60** of the base substance to be transferred to the aqueous bath **18**. This increases the pH to maintain the pH within the desired range.

In certain alternative embodiments of the invention, regions on the metal component **12** may be masked with a protective coating to prevent contact with, or wetting by, the aqueous bath **18**. In particular, regions on metal component **12** that are not coated by coating **10** may be covered by the protective coating, which operates as a barrier preventing contact or wetting by the aqueous bath **18**. After the stripping process removes coating **10**, the protective coating is likewise stripped. Certain types of metal components **12** may include an outer paint layer that is removed before the protective coating is applied or the metal component **12** is contacted with the aqueous bath **18** to strip the coating **10**. An exemplary protective coating is a silane, such as BTSE.

U.S. Pat. Nos. 6,294,072, 6,645,365, and 6,837,985, which describe similar apparatus and methods for stripping, are hereby incorporated by reference herein in their entirety.

The stripping apparatus and methods described herein may be employed in a process for stripping diverse coatings present on a collection of parts, such as a collection of different metal components **12** in which the composition of the coating **10** on each component is an unknown or may comprise one of a finite group of known compositions. For example, the composition of the coating **10** on one metal component **12** may be WCCo and the composition of the coating **10** on another metal component **12** may be CrC/NiCr (i.e., W and Co are absent from the coating composition). The diversity of the composition among the different coatings **10** may preclude the use of a universal stripping operation in which all of the components **12** are simultaneously stripped with one aqueous bath **18** and demands instead the use of different stripping conditions to efficiently strip of the different coatings **10**. For example and as discussed elsewhere herein, stripping conditions required to remove CrC/NiCr coatings **10** generally differ from stripping conditions used to remove WCCo coatings **10**. As another example, one or more outer coatings concealing an inner CrC/NiCr or WCCo coating in a multi-layer coating **10** may prevent successful stripping by stripping processes believed suitable to strip CrC/NiCr or WCCo as these outer coatings may not be effectively removed by the stripping processes suitable for CrC/NiCr or WCCo. For example, an outer layer composed of an organic material (e.g., an aluminum/poly resin) and/or a layer of yet a different material, such as the metal nickel (Ni), may be present on a batch of components **12** that includes WCCo as an innermost coating residing on the exterior surface of each component **12**.

In one embodiment, different types of coatings **10** on a group of metal components **12** may be differentiated and then the metal components **12** sorted by coating type for different stripping processes. For example, the coatings **10** on a group of metal components **12** may be analyzed with a technique

## 13

that elementally identifies one or more primary elements present in the layer(s) of the coating **10**. If the coating **10** consists of a single layer, then one or more elements in the coating **10** may be identified by the elemental analysis. If the coating **10** contains multiple layers, then one or more elements in the outermost layer of the coating **10** may be identified by the elemental analysis. Alternatively, the analytical technique may penetrate through the outermost layer to sample the composition of one or more of the inner layers of coating **10** either in addition to, or instead of, the outermost layer. The same effect may be observed if the outer most layer(s) are not continuous so that various different layers in the stack are exposed during the analytical measurement.

One suitable analytical technique is x-ray fluorescence (XRF), which excites a material high-energy X-ray bombardment and observes the characteristic secondary (or fluorescent) X-ray emission. For example, the wavelengths of the primary spectral lines that may be useful in distinguishing WCCo from CrC/NiCr are a  $K\alpha_1$  line at 0.1789 nm for Co, an  $L\alpha_1$  spectral line at 0.1476 nm for W, and a  $K\alpha_1$  spectral line at 0.1658 nm for Ni. In a batch of components **12** known to be coated with either WCCo or CrC/NiCr, XRF may be used to quickly discriminate between WCCo from CrC/NiCr based upon the presence or absence of the primary spectral lines for W and Co in the secondary X-ray emission. Components **12** with WCCo coatings **10** are then sorted from components with CrC/NiCr coatings **10** so that different stripping techniques can be applied. As another example, silicon containing coatings **10** may be discriminated from CrC/NiCr coatings **10** through the presence or absence of the  $K\alpha_{1,2}$  spectral line for silicon at 0.7126 nm so that different stripping techniques can be applied to remove the different types of coatings **10**. Portable and handheld XRF instruments are commercially available from various commercial sources and operate to perform elemental analyses as understood by a person having ordinary skill in the art.

After sorting, the components **12** in each sorted group are stripped using a different strip process that optimizes the removal of the observed coating **10**. Based upon the elemental analysis, the components **12** may be sorted into groups and then subjected to different types of stripping processes. The composition of the aqueous bath **18**, in each instance, may be selected to optimize the stripping operation that removes the coatings **10**. Each of the processes may be self-limited by a dramatic reduction in stripping rate at the transition between different sub-layers, or an end point of each process may be detected. In either event, the stripping process is changed or modified as the sub-layers of the coating **10** are successively removed.

In another embodiment, a multi-layered coating **10** with a particular combination of sub-layers may be removed from metal component **12** by a series of diverse processes. The combination of sub-layers in the coating **10** may be known or may be deduced as outlined above using elemental analysis techniques. A stripping process is selected that optimizes the removal of each individual sub-layer. Each of the discrete stripping processes may leave behind debris from the sub-layer on the exterior surface of the metal component **12** in the form of an accumulated residue. Between consecutive processes, the accumulated residue may be removed. For example, the exterior surface of the metal component **12** may be scrubbed with nylon-impregnated abrasive pad to effect removal of the accumulated residue. Reliance upon the abrasive pad eliminates the conventional practice of grit blasting the component to remove the accumulated residue. One such abrasive pad is a Norton Bear-tex® commercially available from McMaster Carr. The abrasive pad may be shaped to promote material removal. The scrubbing process may use a power driven movement (i.e., air motor driven motion) of the abrasive pad to remove the accumulated residue from the

## 14

exterior surface of the metal component **12**. Alternatively, any or all of the individual stripping processes may be interrupted for debris removal at intervals during the process, rather than merely at the conclusion of the process. For example, any or all of the individual stripping processes may be interrupted hourly or at 30 minute intervals to remove the accumulated residue. Removing the accumulated residue during the stripping process may result in faster stripping of the particular coating sublayer. Rather than a driven abrasive pad, a water jet or blast may be used for removal of the accumulated residue.

Specifically, a layer stack consisting of a multiple sub-layers, such as an outer layer composed of an organic material (e.g., an aluminum/poly resin), an inner layer composed of WCCo covering the base metal, and a middle layer composed of yet a different material, such as Ni, intervening between the different inner and outer layers, may be removed by a systematic process. A first step in the process is removing the layer of organic material in the coating **10** by a first stripping process. For example, an organic layer composed of an aluminum/poly resin may be removed using an aqueous bath containing sodium hydroxide (NaOH) as an etchant. In one embodiment, the aqueous bath may contain a solution of 0.5 to 1 molar NaOH either heated or at ambient temperature, and the exposure to the aqueous bath may last for two to six hours. Then, the intervening layer in the coating **10** is removed by, for example, an acid etch process. If the middle layer is composed of Ni (e.g., Ni 200), then a heated 10% by volume solution of nitric acid may be used in the stripping operation, and the exposure to the aqueous bath may last for two to six hours. Finally, the inner layer of WCCo in the coating may be removed using an aqueous bath containing citric acid and hydrogen peroxide, as described elsewhere herein. The component **10** may be rinsed before initiating a different stripping process and the accumulated residue may be removed during and/or at the conclusion of each stripping process.

While the invention has been illustrated by the description of an embodiment thereof and specific examples, and while the embodiment has been described in considerable detail, it is not intended to restrict or in any way limit the scope of the appended claims to such detail. Additional advantages and modifications will readily appear to those skilled in the art. For example, a person of ordinary skill in the art will appreciate that general coatings may be stripped from other types of metal components using a stripping apparatus including the concentration sensor, as described herein, and that this aspect of the invention is not limited to stripping coatings from metal components of landing gears and exhaust augmentor flaps. The invention in its broader aspects is therefore not limited to the specific details, representative apparatus and methods and illustrative examples shown and described. Accordingly, departures may be made from such details without departing from the scope or spirit of applicant's general inventive concept.

55 What is claimed is:

1. A method for removing a coating including an outer layer and an inner layer between the outer layer and an underlying metal component, the method comprising:

removing the outer layer of the coating with a first stripping 60 operation by contacting the outer layer with a first aqueous bath;

removing the inner layer of the coating with a second stripping operation by contacting the inner layer with a second aqueous bath that is chemically different from the first aqueous bath, the second aqueous bath having a composition that includes water, an active oxygen source, and a ligand;

## 15

- at least partially removing the coating from the contacted portion of the metal component while the metal component portion is in contact with the second aqueous bath; and
- specifying the first aqueous bath for the first stripping operation based upon an element in the outer layer or the second aqueous bath for the second stripping operation based upon an element in the inner layer.
2. The method of claim 1 wherein specifying the first aqueous bath comprises:
- determining the element contained in the outer layer; and in response to the determination of the element in the outer layer, selecting a composition for the first aqueous bath used in the first stripping operation.
3. The method of claim 2 further comprising:
- determining the element contained in the inner layer; and in response to the determination of the element in the inner layer, selecting a composition for the second aqueous bath used in the second stripping operation to remove the inner layer.
4. The method of claim 3 wherein the element contained in the inner layer is determined after the outer layer is removed.
5. The method of claim 3 wherein the element contained in the outer layer and the element contained in the inner layer are determined by x-ray fluorescence.
6. The method of claim 1 wherein specifying the second aqueous bath comprises:
- determining the element contained in the inner layer; and in response to the determination of the element in the inner layer, selecting a composition for the second aqueous bath used in the second stripping operation to remove the inner layer.
7. The method of claim 6 wherein the element contained in the inner layer is determined after the outer layer is removed.
8. The method of claim 6 wherein the element contained in the inner layer is determined by x-ray fluorescence.
9. The method of claim 1 wherein the active oxygen source is selected from the group consisting of sodium perborate tetrahydrate ( $\text{NaBO}_3 \cdot 4\text{H}_2\text{O}$ ), sodium perborate monohydrate ( $\text{NaBO}_3 \cdot \text{H}_2\text{O}$ ) prepared by dehydrating sodium perborate tetrahydrate, sodium percarbonate ( $\text{Na}_2\text{CO}_3 \cdot 1\frac{1}{2}\text{H}_2\text{O}_2$ ), boric acid ( $\text{H}_3\text{BO}_3$ ), and combinations thereof, and the ligand is selected from the group consisting of citric acid ( $\text{C}_6\text{H}_8\text{O}_7$ ), oxalic acid ( $\text{C}_2\text{H}_2\text{O}_4$ ), tartaric acid ( $\text{C}_4\text{H}_6\text{O}_6$ ), glucose (6-(hydroxymethyl)oxane-2,3,4,5-tetrol), formic acid ( $\text{CH}_2\text{O}_2$ ), and combinations thereof.
10. The method of claim 1 wherein the active oxygen source is hydrogen peroxide ( $\text{H}_2\text{O}_2$ ), and the ligand is selected from the group consisting of citric acid ( $\text{C}_6\text{H}_8\text{O}_7$ ), oxalic acid ( $\text{C}_2\text{H}_2\text{O}_4$ ), tartaric acid ( $\text{C}_4\text{H}_6\text{O}_6$ ), glucose (6-(hydroxymethyl)oxane-2,3,4,5-tetrol), or formic acid ( $\text{CH}_2\text{O}_2$ ).
11. The method of claim 1 wherein removing the outer layer of the coating comprises:
- interrupting the first stripping operation to remove accumulated residue originating from the outer layer.
12. The method of claim 11 wherein removing the inner layer of the coating comprises:
- interrupting the second stripping operation to remove accumulated residue originating from the inner layer.

## 16

13. The method of claim 1 wherein removing the inner layer of the coating comprises:
- interrupting the second stripping operation to remove accumulated residue originating from the inner layer.
14. The method of claim 1 further comprising:
- after removing the outer layer, removing accumulated residue originating from the outer layer.
15. The method of claim 14 further comprising:
- after removing the inner layer, removing accumulated residue originating from the inner layer.
16. The method of claim 15 wherein the accumulated residue from the outer layer is removed without grit blasting.
17. The method of claim 1 further comprising:
- after removing the inner layer, removing accumulated residue originating from the inner layer.
18. The method of claim 17 wherein the accumulated residue is removed without grit blasting.
19. The method of claim 1 wherein the inner layer is disposed in direct contact with a base metal of the metal component.
20. The method of claim 1 wherein the element in the outer layer is chemically different from the element in the inner layer.
21. A method for removing a coating from an underlying metal component, the coating including an outer layer composed of aluminum polyester resin, an inner layer, and an intermediate layer composed of Ni between the outer layer and inner layer, the method comprising:
- removing the outer layer of the coating with an aqueous bath containing NaOH;
- removing the intermediate layer with an aqueous bath containing dilute nitric acid; and
- after the outer layer and the intermediate layer are removed, removing the inner layer of the coating.
22. The method of claim 21 wherein the inner layer is composed of WCCo, and removing the inner layer comprises:
- contacting the metal component with an aqueous bath having a composition that includes water, hydrogen peroxide ( $\text{H}_2\text{O}_2$ ), and citric acid ( $\text{C}_6\text{H}_8\text{O}_7$ ).
23. A method for removing a coating including an outer layer and an inner layer between the outer layer and an underlying metal component, the method comprising:
- removing the outer layer of the coating with a first stripping operation by contacting the outer layer with a first aqueous bath;
- removing the inner layer of the coating with a second stripping operation by contacting the inner layer with a second aqueous bath that is chemically different from the first aqueous bath; and
- specifying the first aqueous bath for the first stripping operation based upon an element in the outer layer or the second aqueous bath for the second stripping operation based upon an element in the inner layer;
- wherein the outer layer of the coating is composed of an organic material.
24. The method of claim 23 wherein the first aqueous bath contains NaOH.
25. The method of claim 23 wherein the inner layer contains a metal-bonded carbide and the second aqueous bath contains citric acid and hydrogen peroxide.

\* \* \* \* \*

UNITED STATES PATENT AND TRADEMARK OFFICE  
**CERTIFICATE OF CORRECTION**

PATENT NO. : 8,377,324 B2  
APPLICATION NO. : 12/415492  
DATED : February 19, 2013  
INVENTOR(S) : David C. Fairbourn

Page 1 of 1

It is certified that error appears in the above-identified patent and that said Letters Patent is hereby corrected as shown below:

In the Claims:

Column 15, line 51, **Claim 10**, change “(hydroxymethyl)oxane2,3,4,5-tetrol),” to  
-- (hydroxymethyl)oxane-2,3,4,5-tetrol), --

Signed and Sealed this  
Seventeenth Day of September, 2013



Teresa Stanek Rea  
Deputy Director of the United States Patent and Trademark Office